

## UNITED STATES PATENT OFFICE

LOCKWOOD W. FERRIS, OF SALT LAKE CITY, UTAH

## PREPARING OXIDIZED MINERALS FOR CONCENTRATION BY FROTH FLOTATION

No Drawing.

Application filed March 31, 1930. Serial No. 440,621.

This invention relates to a method of preparing oxidized minerals for concentration by froth flotation, and its principal object is to render amenable to concentration by froth flotation, certain oxidized minerals which it has been heretofore either impossible to treat, or possible only with difficulty, by means of froth flotation.

I have discovered that by the use of various compounds of thiocarbonic acid, oxidized minerals, such as lead carbonate, lead sulfate, lead oxides, lead molybdate, and other non-sulfide lead compounds, also, such as copper carbonate, copper silicate, metallic copper, and other non-sulfide copper minerals, may be so conditioned that they are often amenable to concentration by froth flotation, whereas, without the use of some thiocarbonic acid compound, such minerals cannot be so concentrated, or else present difficulties to such concentration.

It is to be clearly understood that the present method contemplates the use of compounds of thiocarbonic acid solely to condition the mineral particles for flotation, the actual flotation being accomplished by means of one or more actual flotation agents, such as an oil, amyl xanthate, and so on.

It should be clear that the thiocarbonic acid radical is the agent which creates the desired condition. Inasmuch as thiocarbonic acid itself is unstable and difficult to manufacture, its most convenient form is either as a metallic salt, such as sodium thiocarbonate, potassium thiocarbonate, and so on, or an organic salt, such as ethyl thiocarbonate, amyl thiocarbonate, and so on.

Owing to its convenience, I have preferred to use sodium tri-thiocarbonate, a reaction product between sodium sulfide and carbon bisulfide, as indicated by the following equation:  $\text{Na}_2\text{S}$  plus  $\text{CS}_2$  equals  $\text{Na}_2\text{CS}_3$ .

Sulfur may be dissolved in the sodium sulfide, thus making a sodium polysulfide, which gives a better reaction with the carbon

bisulfide than does the normal sodium sulfide.

In practicing my improved method, the flotation pulp may be prepared in any usual manner, and be aerated or agitated in any suitable flotation machine. The thiocarbonic acid compound may be added to the flotation pulp at any suitable stage of the ordinary process of flotation, that is to say, either before, at the beginning of, or during agitation or aeration of the pulp.

The amount of thiocarbonic acid and/or compounds thereof, used in my process, depends upon the nature of the particular ore being treated. The relative quantities that may be used, are best illustrated by examples from actual practice. Therefore, I give below the results obtained in the treatment of three ores of different character. These examples are:

(a) An oxidized ore from Arizona, carrying about two per cent copper, mostly in the form of silicate:

|                           | Assay per cent copper | Percent total copper | 70 |
|---------------------------|-----------------------|----------------------|----|
| Tails.....                | 0.48                  | 18.2                 |    |
| Cleaner tails.....        | 1.28                  | 23.2                 |    |
| Cleaner concentrates..... | 20.6                  | 58.6                 |    |
|                           |                       | 100.0                | 75 |

## Reagents used per ton of ore

1.0 lb. sodium tri-thiocarbonate.  
0.5 lb. amyl xanthate.  
0.1 lb. frothing agent.

(b) An ore from Mason Valley, Nevada, carrying about 1.3 per cent copper in the form of a mixture of copper carbonate and copper silicate:

## Assay per cent copper

|                           |       |
|---------------------------|-------|
| Tails.....                | 0.025 |
| Cleaner tails.....        | 0.10  |
| Cleaner concentrates..... | 20.6  |

*Reagents per ton of ore*

1.0 lb. sodium trithiocarbonate.

1.0 lb. amyl xanthate.

0.2 lb. frothing agent.

5

(c) An oxidized ore from the Yellow Pine  
mine at Goodsprings, Nevada:

| 10                        | Assay<br>per cent<br>lead | Percent<br>total<br>lead |
|---------------------------|---------------------------|--------------------------|
| Tails.....                | 0.17                      | 2.9                      |
| Cleaner tails.....        | 11.9                      | 31.6                     |
| Cleaner concentrates..... | 40.3                      | 65.5                     |
|                           |                           | 100.0                    |
| 15                        |                           |                          |

*Reagents used per ton of ore*

3.0 lbs. sodium silicate.

2.0 lbs. sodium trithiocarbonate.

20 2.0 lbs. amyl xanthate.

0.1 lb. frothing agent.

In Example (a), the results obtained by  
means of the present process, indicate a re-  
covery of 81.8 per cent; in Example (b), a  
recovery of 95.5%; and in Example (c), a  
recovery of 97.1%.Having fully described my invention, what  
I claim is:30 1. In the concentration of oxidized ores  
by froth flotation, the improvement which  
comprises subjecting the ore in the form of  
a pulp to the action of an alkali-metal tri-  
thiocarbonate.35 2. In the concentration of oxidized ores  
by froth flotation, the improvement which  
comprises subjecting the ore in the form of  
a pulp to the action of sodium trithiocar-  
bonate.40 3. In the concentration by froth flotation  
of oxidized ores containing silicate and car-  
bonate minerals, the improvement which  
comprises subjecting the ore in the form of  
a pulp to the action of sodium trithiocar-  
bonate.45 4. In the concentration by froth flotation  
of oxidized ores containing carbonate min-  
erals, the improvement which comprises sub-  
jecting the ore in the form of a pulp to the  
action of an alkali metal trithiocarbonate.50 5. In the concentration by froth flotation  
of oxidized ores containing carbonate min-  
erals, the improvement which comprises sub-  
jecting the ore in the form of a pulp to the  
action of sodium trithiocarbonate.55 In testimony whereof, I sign my name  
hereto.

LOCKWOOD W. FERRIS.